

Oct. 30, 1928.

1,689,311

E. B. WHEELER

INSULATED WIRE

Filed Oct. 9, 1924



Inventor:  
Edmund B. Wheeler  
by *Sw. Adams* Atty.

## UNITED STATES PATENT OFFICE.

EDMUND B. WHEELER, OF NEW YORK, N. Y., ASSIGNOR TO WESTERN ELECTRIC COMPANY, INCORPORATED, OF NEW YORK, N. Y., A CORPORATION OF NEW YORK.

## INSULATED WIRE.

Application filed October 9, 1924. Serial No. 742,498.

This invention relates to electrically insulated wire and particularly to so-called "flame-proof" electrically insulated wire.

An object of the invention is to provide a covering for a wire which shall be substantially flame-proof as well as an efficient insulator or non-conductor of electricity.

A feature of the invention is a wire having a coating thereover comprising selenium and cellulose acetate.

A further feature is a wire having an insulating covering and a coating thereover containing selenium and cellulose acetate.

A further feature is a wire having an insulating covering, a coating comprising selenium and cellulose acetate over the insulating covering, and an exterior textile covering.

A further feature is a wire having an insulating covering, a coating of finely-divided selenium and cellulose acetate over the insulating covering, and an exterior covering of flame-proofed cotton.

The single figure of the drawing shows an insulated wire embodying one form of the invention.

Referring to the figure, the insulated wire comprises a core 1 of electrically-conducting material, a coating 2 of insulating material applied over the core 1, a second coating 3 of flame-proof material comprising finely-divided selenium and cellulose acetate over the insulated covering 2, and an exterior textile covering 4, such as cotton or flame-proofed cotton, applied over the flame-proof coating 3.

One way of producing the flame-proof insulated wire embodying the invention is to pass a wire of electrically conducting material which may have an insulation covering, such as rubber, rubber compounds or enamel, through a bath containing a solution of cellulose acetate lacquer having finely-divided selenium in suspension therein, the solution being of the proper consistency to give the required thickness of coating. The cellulose acetate lacquer may comprise cellulose acetate dissolved in a suitable solvent, such as acetone. The wire may be drawn through the solution in any suitable manner, but preferably should be drawn out of the solution in a vertical direction so as to obtain a coating of uniform thickness around the wire. When

the wire is withdrawn from the solution, after a short interval of drying in air, which may be heated, the lacquer solvent will evaporate and a uniform coating 3 of dried or partially dried mixture comprising finely-divided selenium and cellulose acetate will be obtained on the insulated wire.

A very small amount of the finely-divided selenium mixed with the cellulose acetate lacquer will give very effective flame-proofing.

When heat is applied to the wire, the selenium powder, apparently, acts as a rapid de-oxidizer, thus maintaining the insulated conductor beneath in an inert atmosphere and making it resistant to flame. Cellulose acetate has several properties which make its use especially advantageous on insulated wire.

Because of its good adhesive qualities, the cellulose acetate lacquer makes a satisfactory binding medium for the finely-divided selenium and gives a coating which will have sufficient flexibility and adherence to permit reeling and considerable handling;

the cellulose acetate lacquer dries quickly which is a manufacturing advantage; in itself, cellulose acetate is an effective insulator and non-conductor of electricity; it is not hygroscopic and therefore the insulation resistance remains high under varying atmospheric conditions, and the covering also provides considerable water-proofing; and it is relatively non-combustible and therefore gives additional flame-proofing other than that obtained from the finely-divided selenium.

The flame-proofing coating comprising finely-divided selenium and cellulose acetate may be further protected from abrasion by applying an outer textile covering or serving 4, preferably of cotton or cotton braid, over it by processes well known in the art, and an additional flame-proof and water-proof protection may be obtained by impregnating the textile fabric with any suitable flame-proofing material, for example with sodium-magnesium borate.

If desired, the textile covering 4 may be applied before the coating containing cellulose acetate has dried, so that the coating in its liquid or partially set condition is taken up to some extent by the covering thus improving the adherence between the covering and

the insulated conductor. In either case, the finely-divided selenium and the cellulose acetate are given further protection from abrasion by the covering. A practically continuous coating of the flame-proof material is thus maintained over the insulation coating.

The wire produced as above described is found to be an efficient flame-proof conductor which may be used in any situation where 10 flame-proofing is necessary.

What is claimed is:

1. Means for flame-proofing a conductor comprising a coating of finely-divided selenium and cellulose acetate.
- 15 2. An insulated wire comprising a core of electrically conducting material having a coating of insulating material, and a second coating comprising selenium and cellulose acetate over the first mentioned coating to 20 make the insulated wire less flammable.
- 20 3. An insulated wire comprising an electrically conducting core having a coating of insulating material, a second coating comprising selenium powder and cellulose acetate applied

over said first mentioned coating, and a textile covering over said second coating.

4. An insulated wire comprising a core of electrically conducting material having a coating of insulating material thereover, a second coating comprising selenium powder 30 and cellulose acetate applied over said first mentioned coating, and a cotton covering impregnated with flame-proofing material applied over said second coating.

5. A wire having an electrical insulation of 35 rubber, a flame-proof insulation of powdered selenium and cellulose acetate applied over the rubber, and a mechanical insulation of closely woven cotton applied over said flame-insulation.

6. A flame-proof insulation for electrical conductors, comprising a coating of cellulose acetate having finely divided selenium suspended therein.

In witness whereof, I hereunto subscribe 45 my name this 29th day of September A. D., 1924.

EDMUND B. WHEELER.